

Dec. 26, 1922.

1,439,937

C. A. BACON.  
CHILLED MOLDBOARD AND POINT FOR PLOWS AND THE METHOD OF MAKING SAME.  
FILED MAR. 29, 1920.



Fig. 1



Fig. 2



Fig. 3



Fig. 4

WITNESS:  
Wm Casati

INVENTOR.  
Charles Allen Bacon,  
BY  
Arthur L. Sprinkle,  
ATTORNEY.

## UNITED STATES PATENT OFFICE.

CHARLES ALLEN BACON, OF SOUTH BEND, INDIANA.

## CHILLED MOLDBOARD AND POINT FOR PLOWS AND THE METHOD OF MAKING SAME.

Application filed March 29, 1920. Serial No. 369,466.

*To all whom it may concern:*

Be it known that I, CHARLES ALLEN BACON, a citizen of the United States, residing at South Bend, in the county of St.

5 Joseph and State of Indiana, have invented certain new and useful Improvements in Chilled Moldboards and Points for Plows and the Method of Making Same, of which the following is a specification.

10 The invention relates to an article of manufacture comprising mold board and point for plows and the method of making same, and has for its object to produce a mold board and point for plows in which 15 the operative surfaces thereof shall be constructed of chilled cast metal, but in which there shall be an interior or inner stratum of a tough and softer metal as steel of a low carbon content, the improved method being 20 designed to permit the operative and wearing surfaces of both mold board and point to be formed of cast chilled metal united with the said inner stratum of tougher metal of low carbon content, which is a result not 25 heretofore attained in the manufacture of mold boards and points for plows.

Other objects of the invention will appear from the following description, which is directed to the preferred embodiment as hereinafter described and claimed, and illustrated as far as possible in the drawing which forms a part of the specification.

In the said drawing, Fig. 1 is a view in side elevation of a mold board and point of 35 conventional form illustrating the manner in which the soft metal inner stratum appears when cast in the chilled mold board or point.

Fig. 2 is a detail sectional view through 40 the mold board on line 2—2 of Fig. 1, looking in the direction indicated by the arrows, and showing the relative arrangement of the outer chilled strata of metal and the inner or intermediate stratum of tough metal of low 45 carbon content.

Fig. 3 is a sectional view similar to Fig. 2, being taken through the plow point on line 3—3 of Fig. 1.

Fig. 4 is an illustrative view showing a 50 flask in section in which a mold board may be formed or cast in accordance with the method of the invention, the flask itself being shown in section as well as the metallic hollow steam heated chill. In this view the 55 intermediate stratum of metal of low carbon content is shown in position in the flask

to receive the metal forming the outer strata of a chilled mold board or point in carrying out the method embodying the invention.

It is well recognized in the art of manufacturing agricultural implements such as plows, that it is desirable to provide the wearing surfaces of the points or shares and mold boards with hardened chilled surfaces wherever such surfaces come in direct contact with the earth, and this is particularly desirable in sandy soils on account of the well known abrasive effect of sand and small rock particles upon the metal. For this reason it has been common heretofore to construct mold boards and points or shares for plows either of hardened or chilled cast metal or when it has been desired to form the shares or points and mold boards of rolled metal as steel, it has been 70 proposed to form a composite member for the points and mold boards by rolling together sheets of steel of high carbon content on the outer surface with an inner stratum of a tougher metal as steel of low 80 carbon content. Certain advantages however, are inherent in cast mold boards and points for certain conditions of soil over any rolled or otherwise forged and mechanically formed and tempered metallic points and 85 mold boards. Therefore it has been the aim of the present improvement to combine in a cast chilled mold board and point all the advantages of mold boards and points as heretofore rolled or forged and hardened without having any disadvantages of the latter.

In carrying out my invention in the formation of mold boards and points for plows, I first form the inner stratum of ductile or tough metal as steel of low carbon content in substantially the form or outline of the completed mold board or point, as illustrated for example in Fig. 1, by the dotted line, it being the intention that this inner stratum shall extend for strengthening 100 purposes substantially throughout the completed mold board and point, as will be seen from an inspection of the indicated inner stratum, as shown in Fig. 1 and as illustrated also in section through the mold 105 board and point respectively in Figs. 2 and 3. The reference character 10 is used generally to indicate the mold board and reference character 11 is applied generally to the point or share of the plow. Reference 110 characters *a* and *b* indicate the inserts or inner stratum of the mold board and point

or share respectively. Obviously, the invention may be applied to the production of mold boards and points of any desired configuration and from an inspection of the 5 sectional views of mold board and point or share respectively, as shown in Figs. 2 and 3, it will be seen that on the exterior of the inner strata *a* and *b* of tough ductile steel of low carbon content, I form a coating 10 of cast chilled metal, preferably on both sides of the inner plates *a* and *b*, although my chief concern is to determine that the normal outer or wearing surface of the mold board shall be properly chilled as 15 well as the outer or wearing surfaces of the points or shares. Some chilling and consequent hardening of the strata on the opposite sides of both point and mold board will occur in practice on account of the 20 contact of the molten metal with the insert or inner stratum of metal of low carbon content in the casting operation, so that substantially all of the outer and exposed surfaces of both mold boards and points 25 when constructed in accordance with the principles of the invention will be of chilled hardened metal. The details of the preferred method of practicing the invention will be made apparent from the following description, with particular reference to Fig. 4, from which it will be seen that a flask or casting frame is provided of the usual two-part form, in which the lower frame or drag, which may be of 30 hollow metal, contains a hollow member of metal, which is designated in Fig. 4 by reference character *d*. This hollow member or chill *d* is shown provided with a steam supply pipe *e* connecting with its 35 hollow interior for warming same to control the temperature thereof, and hence to control the resulting chill imparted to the molten metal poured into the flask in casting. The upper part of the casting frame 40 or flask, commonly called the cope, is designated by reference character 15, while reference character 14 is applied to the lower part thereof. The exposed upper surface of the chill *d* will obviously conform 45 to the wearing surface of either the mold board or plow point or share, as the case may be; although the chill *d* of Fig. 4 is particularly intended for casting mold boards, and in casting points I find that 50 55 efficient chill may be imparted to the resulting product by the introduction of a non-steam heated metallic chill of simple form, if desired. In casting mold boards, however, the steam heated chill is preferable.

The inner stratum of steel of low carbon content used in forming mold boards is illustrated in Fig. 4 as in proper position in the mold cavity for the flask to receive 60 the molten metal as designated in

the drawings by reference character *a*. It will be seen from an inspection of this part in Fig. 4 that plate *a* is suspended within the recess formed by the mold in the flask when assembled. The flask may 70 be of the form commonly used in foundry practice as indicated, consisting of the two parts 14 and 15, and the interior mold will be formed by the introduction of the pattern and the subsequent granular material 75 of sand to form the mold. After the separation of the flask and the removal of the pattern the stratum or plate of tough metal of low carbon content *a* will be introduced into the mold cavity and will be held in its 80 proper position to permit the flow of the molten chilled cast metal on both sides thereof, as illustrated in Fig. 4. Any suitable means may be employed to position the inner plate or stratum *a* within the mold 85 cavity prior to the introduction of the molten metal to complete the mold board or point.

One method of positioning the plates *a* in the mold used by me has been to suspend the plates from wires held in the upper section or cope of the mold. The reference character 20 designates one of such hooked wires fastened in the cope as indicated at the right end of Fig. 4. Obviously, 90 if such be used a plurality will be required around the periphery of the plate *a* when in position in the mold. Upon the introduction of the molten metal such wires will serve the purpose of retaining the plate in 95 proper position until it will be held by the cooling and chilling of the molten metal, which at the same time will result in melting the wire and amalgamating same with the metal of the resulting product.

Another method I have employed successfully in positioning the inner stratum plates *a* in the mold cavity consists of small blocks or portions of metal all substantially the same quality as used in casting the outer 110 strata of the mold board or point. A plurality of these may be scattered over the upper exposed surface of the chill *d* of the desired thickness to properly position the plate *a*. Upon the introduction of the molten metal these obviously, will be amalgamated with the resulting casting if they be formed of sufficiently small body. After the inner strata of plates *a* and *b* are in position, as indicated by the position of plate *a* in Fig. 4, the mold is in condition 115 for the pouring of the molten material to form the casting, which may be introduced in the conventional manner through an opening in the mold, as indicated by reference character 24, the same extending downwardly through cope and drag to the mold cavity at one of the lateral edges, it being preferred that the orifice leading to the cavity shall permit the entry of metal 120 125 130

throughout the entire thickness of the cavity so that the metal will flow freely into the mold cavity and directly on top of the chill as well as on the top side of the mold cavity, 5 and consequently, on the upper side of the inner stratum or plates *a* and *b*.

In order to insure the best union or contact between the strata of the composite mold boards or points formed according to 10 the principles of the invention, I follow the practice of immersing or pickling the inner stratum plates *a* and *b* in a suitable acid solution, as well known in the art, to remove foreign particles and to roughen the 15 surface. In order to further insure an inseparable union between the strata of the completed product, I prefer to form also especially in plates *a* of the mold board a number of comparatively small perforations, as indicated by reference character *g*, 20 Fig. 1. Obviously, the molten metal forming the outer strata of the mold board in flowing along both top and bottom side of the plate will pass through such perforations and meet, thus more firmly locking the inner stratum plates *a* and *b* in the resulting product. After the casting operation, as described, takes place, no other special steps are necessary, the mold boards and 25 points being simply removed from the flasks and treated as ordinary chilled cast mold boards and points to put them in condition for commercial usage on the plow.

In practicing the above described method 30 in the formation of chilled mold board and point castings I have found that the operative surfaces of the castings come from the molds in a more perfect condition than in the ordinary chilled casting operations heretofore employed, this condition being more 35 perfect with respect to smoothness as well as harder, and such hardness is of a more uniform character than in chilled mold boards as cast by heretofore common practice. 40

Another important result attained in mold boards and points cast by my improved process results from the fact that with the steel centers of low carbon content, although the outer and wearing surfaces are of a 50 harder character and more uniform with respect to this quality, they are also found to resist fracture or breakage to a much greater extent than in mold boards and points of a corresponding thickness formed 55 of chilled cast metal throughout. Tests on mold boards and points made according to the method herein described indicate to me that a mold board or point made in accordance with my invention will resist breakage 60 to approximately the same extent as the average soft center steel mold board.

In order that the invention might be understood I have described the preferred manner of practicing the invention, but it 65 is not desired to be limited to the precise details set forth, for it is apparent that persons skilled in this art may secure the benefits of the invention and yet vary to a considerable extent the details thereof, as 70 herein set forth.

I claim:

The herein described method of making mold boards and points for plow bottoms which consists in positioning in a mold cavity 75 an inner stratum sheet of the general form of the mold board or point, said inner stratum sheet consisting of steel of low carbon content, and subsequently admitting to the interior of the mold molten metal to 80 form a stratum or covering over said inner stratum sheet, the said covering or stratum being subjected in the mold to means for chilling and hardening the exterior surface thereof.

In testimony whereof I have signed my 85 name to this specification, on this 17th day of March, A. D. 1920.

CHARLES ALLEN BACON.